

June 22, 1926.

1,589,513

A. L. CLAPP

METHOD AND MACHINE FOR MAKING FIBER BOARD OF VARIABLE THICKNESS

Filed March 7, 1924



Patented June 22, 1926.

1,589,513

# UNITED STATES PATENT OFFICE.

ALBERT L. CLAPP, OF DANVERS, MASSACHUSETTS, ASSIGNOR TO THE FLINTKOTE COMPANY, OF BOSTON, MASSACHUSETTS, A CORPORATION OF MASSACHUSETTS.

## METHOD AND MACHINE FOR MAKING FIBER BOARD OF VARIABLE THICKNESS.

Application filed March 7, 1924. Serial No. 697,487.

Roofing material as now commonly made from felted fibrous material, such as rag felt saturated with waterproofing material as asphalt, with or without a surfacing of 5 granular material, as crushed slate, is of substantially uniform thickness. Where such material is laid in overlapping courses it must be somewhat flexible in order to lie tight to the roof, the upper edge of each 10 course engaging the roof foundation and then bending up and over the upper edge of the underlying course and then flat against its upper face. In order that substantially rigid roofing elements, such for example as 15 wood shingles, may be laid in overlapping courses and lie flat, it is necessary to form them tapering in thickness, the thin edges being uppermost forming no sudden rises over which the units of the overlying course 20 must pass and then be bent down to lie flat against the upper faces of the underlying units. As ordinarily constructed a paper machine is incapable of forming sheet material tapered in thickness and hence 25 heretofore it has been necessary where roofing material is to be formed on a paper machine to form this material flexible. Flexible material, however, has the disadvantage that the portion exposed to the 30 weather is liable to be bent upwardly, permitting rain to drive up under and impairing its weatherproofing capabilities.

This invention, therefore, provides a method and machine by which a relatively 35 stiff waterproof board, such for example, as that described and claimed in my application, Serial No. 662,225, filed September 12, 1923 for shingle material and method of manufacture, may be formed tapered in 40 thickness on a wet paper machine so that it is well adapted for weatherproofing purposes and may be laid flat in the same manner as ordinary tapered wood shingles.

This may be accomplished by removing 45 portions of the pulp variable in longitudinal extent across the width of the web of the pulp picked up by the take-up roll so that the amount of pulp deposited on the make-up roll is variable axially to produce the 50 desired taper in the finished board.

For a more complete understanding of this invention reference may be had to the accompanying drawings in which

Figure 1 illustrates diagrammatically in

plan a wet paper machine designed to form 55 the board in the manner above set forth.

Figure 1<sup>a</sup> illustrates in an exaggerated degree the varying cross section of the pulp as deposited on the make up roll.

Figure 2 represents a diagrammatic side 60 elevation of the same.

Figure 3 is a section through the make up roll and a portion of the end couch roll over which the blanket of the paper machine passes, these rolls being constructed to 65 form the board tapered.

Figure 4 represents the board as taken from the make up roll cut through at its portions of greatest and least thickness preparatory to being cut crosswise into shingle 70 units.

Referring first to Figures 1 and 2, at 1 is indicated diagrammatically the vat of a paper machine in which revolves the usual cylinder mold 2, over which passes the 75 blanket or felt 3 on which the pulp picked up by the mold 2 is deposited, the blanket passing over the rear couch roll 4 so that the felted fiber deposited on the blanket from the cylinder mold lies on the upper 80 side of the blanket in the form of a continuous web of substantially uniform thickness in the usual manner. Provision is then made by which portions of the pulp are removed from the blanket periodically, these 85 portions extending throughout a portion of the width of the web only and being spaced at intervals lengthwise thereof. Where the web is unbroken, therefore, it will be evident that all the pulp picked up is deposited on 90 the make up roll and in zones laterally of the web where some of the pulp has been removed, less pulp will be deposited on the make up roll so that the board will be thinner 95 at these zones than where the web is uninterrupted as shown in Figure 1<sup>a</sup>.

Means for removing the pulp from the blanket in the desired zones may comprise rollers, such as shown at 6 and 7 in Figures 1 and 2. As shown the roller 6 comprises 100 four spaced portions 8 of comparatively large diameter joined by intermediate portions 9 of smaller diameter. This roll is positioned above the blanket which may be supported beneath by a roller of uniform diameter as 105 at 10 over which it passes. The roller 6 is mounted so that it may be permitted to drop against the web of pulp traveling therebe-

neath on the blanket, the portions 8 thereof contacting with the pulp which is picked up thereon in spaced zones each of a width of the axial dimension of the corresponding portion 8, and of a length depending on the time during which the roller 6 is allowed to be in depressed position. When the roller 6 is raised, the portions 8 are moved from contact with the pulp which thereupon continues to move in an uninterrupted web toward the make up roll. As shown the roller 6 is journaled at the ends of a pair of arms 12 pivoted at 13 and these arms may be rocked upwardly to remove the roller from contact with the web by means of a cam 15 carried by a shaft 16, the cam engaging a follower 17 at the lower end of a push rod 18 having its upper end connected to one of the arms 12. The cam is so formed as to permit the roller 6 to be dropped into contact with the web during the desired time intervals to remove the pulp from the web in spaced zones laterally thereof in definite lengths, the roll being raised between these time intervals to permit the web to pass uninterrupted. As herein shown the roller 6 is permitted to engage the web to remove portions thereof during substantially one-third of the time the web is passing therebeneath so that substantially one-third of the material is removed from the web in zones corresponding to the positions of the portions 8 of the roller.

As herein shown also the roller 7 is provided with a pair of spaced portions of enlarged diameter 20 corresponding to the spaces between the two outer portions 8 of the roller 6. These portions 20 are allowed to descend into contact with the web to remove pulp therefrom for which purpose the roller 7 is shown as carried by arms 21 which may be raised and permitted to fall by means of a cam 22 in a similar manner to the roll 6. This cam, however, permits the portions 20 to engage the surface of the web over longer time intervals than the portions 8 are permitted to engage it, whereupon more of the pulp is removed in zones spaced laterally of the web corresponding to the positions of the portions 20 than corresponding to the positions of the portions 8. As herein shown substantially two-thirds of the pulp is removed from the web in the lateral zones corresponding to the positions of the portions 20.

The web of pulp having portions of variable extent spaced laterally thereof removed by the action of the rollers 6 and 7 is then carried along by the blanket 3 which passes over the end couch roll 25 over which is positioned the make up roll 26 on to which the pulp in the web is wound, being entirely removed thereby from the blanket. The make up roll is shown in section in Figure 3 and referring to this figure, it will be seen that

it is formed tapering, its outer ends 27 and its central portion 28 being of somewhat smaller diameter than the intermediate portions 29, the roll tapering between these portions. The end couch roll, however, is formed cylindrical so that the blanket passes thereover in the usual manner without being stretched or otherwise distorted, the variations laterally of the web for receiving the pulp being formed entirely on the make up roll. As the make up roll is pressed down against the couch roll under considerable pressure, the pulp deposited thereon in layers of variable thickness axially is reduced to a somewhat gradual taper instead of the stepped formation in which it is deposited as indicated in Figure 1<sup>a</sup>. As there shown the pulp is deposited on the make up roll in zones of different thickness corresponding to positions of the portions 8 and 20 of the rollers 6 and 7 and the portions of the web which are continuous at either end of the end portions 8 and between the central portions 8 where both rollers 7 fail to remove any of the pulp.

The board is removed from the make up roll in the usual manner and is cut through longitudinally of the web to form sections tapered in thickness as shown in Figure 4. These may be subjected to pressure to condense the material into firm rigid tapered boards which may cut through as along the dotted lines 30 shown in Figure 3 to form shingle elements of tapered thickness. The pulp taken up by the rolls 6 and 7 is taken therefrom and returned to the beater as often as may be found desirable.

Having thus described an embodiment of this invention it should be evident that various changes and modifications might be made therein, as for example, more rollers for removing the pulp might be employed to render the pulp deposited on the make up roll of more gradual variable thickness in adjacent zones and various other changes and modifications might suggest themselves to those skilled in the art without departing from the spirit or scope of this invention as defined by the appended claims.

I claim:

1. The method of making a board of variable thickness on a wet paper machine which comprises, removing from the blanket of the machine definite portions of the web of pulp deposited thereon, and collecting the remainder of the pulp deposited on the blanket on a make up roll.

2. The method of making a paper board of variable thickness on a wet paper machine, which comprises removing portions of the web of pulp deposited on the blanket of the machine, the amount removed being progressively variable across the width of the blanket, and collecting the remainder of the pulp so deposited on a make up roll.

3. The method of making a paper board on a wet paper machine, which comprises removing portions of the web of pulp deposited on the blanket of a machine, the amount removed being progressively variable across the width of the blanket, and collecting the remainder of the pulp so deposited on a make up roll, having its periphery formed lengthwise to the desired tapered contour.
4. The method of making a paper board on a wet paper machine, which comprises removing portions of the web of pulp deposited on the blanket of a machine, the amount removed being progressively variable across the width of the blanket, and collecting the remainder of the pulp so deposited on a make up roll, having its periphery formed lengthwise to the desired tapered contour,
- removing the pulp from the make up roll in board form and subjecting the board to pressure.
5. The method of forming a fiber board of variable thickness which comprises forming a web of fibrous pulp, removing therefrom periodically portions of variable lengthwise extent laterally of the web.
6. The method of forming a fiber board of variable thickness which comprises forming a web of fibrous pulp, removing therefrom periodically portions of variable lengthwise extent lengthwise of the web, rolling the remaining portions into a cylinder having a length corresponding to the width of the web, cutting the cylinder lengthwise, and unrolling it to form the board.
7. The method of forming a fiber board tapering in thickness, which comprises forming the fiber in sheet form, periodically removing portions of the sheet of progressively variable lengthwise extent widthwise of the sheet, and forming the remaining portions of the sheet into a board, the thickest portions thereof corresponding to those portions widthwise of the sheet having the least fiber removed.
8. The method of forming a fiber board tapering in thickness, which comprises forming the fiber in sheet form, periodically removing portions of the sheet of progressively variable lengthwise extent widthwise of the sheet, and forming the remaining portions of the sheet into a board, the thickest portions thereof corresponding to those portions widthwise of the sheet having the
- least fiber removed, and subjecting the board to pressure to render the paper uniform.
9. A paper machine comprising a vat, a pick-up roll therein, a blanket to receive the layer of pulp picked up by the pick-up roll, a make up roll to receive the pulp from the blanket, and means for periodically removing portions of the pulp in zones laterally of the blanket, whereby the pulp deposited on the make up roll varies in thickness lengthwise thereof.
10. A paper machine comprising a vat, a pick-up roll therein, a blanket to receive the layer of pulp picked up by the pick-up roll, a make up roll to receive the pulp from the blanket, and rollers constructed and arranged to be moved into contact with the pulp on said blanket to remove it therefrom in laterally spaced zones and to definite extent, whereby the pulp deposited on the make up roll varies in thickness lengthwise thereof.
11. A paper machine comprising a vat, a pick-up roll therein, a blanket for receiving a layer of pulp from the pick-up roll, a make up roll for receiving the pulp from the blanket and forming it to the desired thickness, and means for causing the pulp to be unequally spread on the blanket laterally thereof in advance of the make up roll, whereby it is formed of variable caliper on the make up roll lengthwise thereof.
12. A paper machine comprising a vat, a pick-up roll therein, a blanket for receiving a layer of pulp from the pick-up roll, a make up roll for receiving the pulp from the blanket and forming it to the desired thickness, and means for causing the pulp to be unequally spread on the blanket laterally thereof in advance of the make up roll, whereby it is formed of variable caliper on the make up roll lengthwise thereof, the diameter of said make up roll being variable lengthwise complementary to the desired variations in caliper of the board.
13. In a paper machine, a blanket, a pulp roll of uniform diameter over which the blanket of the machine passes, and a make up roll of variable diameter lengthwise thereof arranged to receive pulp non-uniformly deposited across the width of said blanket.

In testimony whereof I have affixed my signature.

ALBERT L. CLAPP.